

## 1

3,577,248

### LOW MOLECULAR WEIGHT LINEAR ALKYL BENZENE SULFONATE AS FROTHING AGENTS FOR GYPSUM BOARD MANUFACTURE

Robert B. Doan, Drexel Hill, and Robert C. Taylor, King of Prussia, Pa., assignors to Atlantic Richfield Company, Philadelphia, Pa.

No Drawing. Filed Nov. 6, 1967, Ser. No. 680,989  
Int. Cl. C04b 11/00

U.S. Cl. 106—111

8 Claims 10

#### ABSTRACT OF THE DISCLOSURE

This invention relates to gypsum boards and to a method for producing the board which utilizes as a frothing agent an alkyl benzene sulfonate having a linear secondary alkyl side chain with an average carbon content ranging from 8.5 to 10.5 and a maximum carbon number spread of 8 carbon atoms. Preferably, the average carbon content ranges from 9.5 to 10.5 and the carbon number spread is a maximum of 5 carbon atoms. This frothing agent is generally utilized in amounts ranging from 0.01 to 0.1 part per 100 parts by weight gypsum.

#### BACKGROUND OF INVENTION

In the production of gypsum board a fluid gypsum slurry is spread between two impervious barriers such as paper sheet and the resultant composition is then heated until the free water has evaporated and the gypsum has set. Because of the weight of gypsum it has become the practice in the industry to incorporate air bubbles into the core to lower the density of the final board. This is accomplished by incorporating a froth or foam into the slurry prior to the evaporation of water. The froth is prepared by agitating an aqueous solution of a frothing agent such as rosin soap. Attempts have been made to utilize in commercial operations synthetic detergents such as alkyl benzene sulfonates having alkyl side chains containing from 11 to 13 carbon atoms which have been very successful in other fields such as dishwashing and clothes washing. It was found, however, that the amount and stability of the foam generated by these frothing agents was not sufficient to insure uniform low density throughout the board.

It has now been discovered that alkyl benzene sulfonates having a linear secondary alkyl side chain with an average carbon content ranging from 8.5 to 10.5 and a maximum carbon number spread of eight carbon atoms is superior to other alkyl benzene sulfonates in producing greater amounts of more stable foam in the gypsum slurry. This phenomenon is unexpected since it is well-known in the art that in other detergent applications alkyl benzene sulfonates having alkyl chains of less than eleven carbon atoms exhibit poorer detergent properties including foam generation and stability. Because of the outstanding stability a substantial portion of the foam remains intact during the agitation and setting of the gypsum slurry in the gypsum board thus permitting the utilization of smaller amounts of foam and consequently lower frothing agent loadings.

It is an object of this invention to provide an improved method of producing gypsum board.

## 2

It is a further object of this invention to provide a new light weight gypsum board having uniform density characteristics.

The alkyl benzene sulfonates which can be utilized in the practice of this invention have the following structural formula



wherein R and R' are linear alkyl radicals and the average carbon content of the sum of R and R' ranges from 7.5 to 9.5. X is an alkali metal ion or ammonium. It has been found that while alkyl benzene sulfonates wherein R+R' ranges from 7.5 to 8.5 impart uniform density to the board their efficiency is impaired by the presence of certain accelerators or retarders such as starch. Preferably, therefore, the average carbon content resulting from the sum of R+R' ranges from 8.5 to 9.5 and the maximum carbon number spread is five. The most suitable salt is that in which sodium is the cation.

The alkyl benzene sulfonates of this invention can be prepared by subjecting a linear olefin or a secondary linear alkyl chloride or alcohol and benzene to an alkylation environment in the presence of an alkylation catalyst such as  $\text{AlCl}_3$ , HF,  $\text{H}_2\text{SO}_4$  or  $\text{BF}_3$ . The alkylated benzene can then be sulfonated utilizing re-agents such as sulfuric acid, sulfur trioxide or oleum. The sulfonated portion of the molecule is then neutralized by reaction with an alkali metal compound such as sodium hydroxide or an ammonium compound such as ammonia or ammonium hydroxide.

The light weight gypsum boards of this invention can be prepared by placing a froth-containing gypsum slurry between two impervious barriers and then evaporating the free water to allow the gypsum to set. The slurry is prepared by adding gypsum to water and agitating. The amount of water will vary depending upon the type of gypsum and the strength and density of the desired board. Generally, the water ranges from 60 to 130 parts per 100 parts gypsum. The froth can be generated in the slurry by merely adding a frothing agent and then agitating the mixture until the desired level of foam is produced. Preferably, however, the foam is first prepared and then added to the slurry. The amount of frothing agent utilized depends ultimately upon the desired density of the board. Other factors which dictate the proper frothing agent loading include the type of gypsum, the hardness of the water and the specific foaming properties of the frothing agent. For most commercial operations the amounts of frothing agent ranges from 0.001 to 1 part per 100 parts gypsum. Optimum loadings are usually in the range of 0.01 to 0.1 part per 100 parts gypsum.

After depositing the slurry between two impervious barriers such as paper sheets, the mixture is then subjected to heat usually at about 250° F. to 350° F. to evaporate the water and allow the gypsum to set. Additional components such as builders or stabilizers can be added to the froth to enhance or increase its basic properties. Various commercial methods of producing gypsum board are well-known in the art as exemplified by U.S. Pat. Nos. 2,560,521; 2,432,963; 2,207,339 and 3,343,818 which are hereby incorporated by reference into this specification.

Various additives can also be utilized to aid in the setting. For example, accelerators such as ground gypsum, potassium sulfate or ammonium sulfate can be added to improve setting rates. Additives such as starch or glue can be added to retard setting at the surface of barriers and thus provide a better core-to-barrier bond. Structural elements such as fibers or ground paper can also be incorporated to alter the strength characteristics of the final board. Most additives are utilized in amounts ranging from 0.1 to 2 parts per 100 parts gypsum.

The following examples are given to illustrate specific embodiments of this invention and should not be construed as limitations upon the scope of invention. All parts are by weight. All alkyl benzene sulfonates utilized in the examples were the sodium salts.

The foam tests utilized in these examples have been found by empirical correlation to provide an accurate indication of the suitability of various frothing agents in commercial production of gypsum board. The foam generation versus time test demonstrates the ability of the frothing agent to be utilized as an in situ foam generation source or in the independent generation of foam at speeds which match the rate of gypsum slurry input. The total foam generated is a measure of the efficiency of the frothing agent in generating foam which dictates its feasibility in a commercial operation. The volume of water separated after specified time intervals indicates the stability of the foam which to prevent collapse of the board must remain intact until the gypsum has set sufficiently.

4  
TABLE I

| Formulation No.                                    | 1    | 2                | 3    | 4    | 5    | 6                | 7     |
|----------------------------------------------------|------|------------------|------|------|------|------------------|-------|
| Average No. of carbons in alkyl chain              | 9.0  | 9.4              | 9.5  | 10.3 | 10.4 | 11.3             | 13.0  |
| Actual alkyl chain carbon range                    | 8-10 | ( <sup>1</sup> ) | 9-10 | 9-11 | 9-13 | ( <sup>2</sup> ) | 12-14 |
| Maximum carbon spread                              | 3    | 12               | 2    | 3    | 5    | 4                | 3     |
| Time (sec.) to generate specified amounts of foam: |      |                  |      |      |      |                  |       |
| 500 cc.                                            | 14   | 13               | 12   | 14   | 15   | 61               | >120  |
| 600 cc.                                            | 21   | 22               | 18   | 20   | 21   | 115              | ----- |
| 700 cc.                                            | 44   | 56               | 31   | 34   | 35   | >120             | ----- |
| 800 cc.                                            | 120  | >120             | 94   | 64   | 87   | -----            | ----- |
| Total foam after 120 seconds                       | 800  | 750              | 815  | 900  | 850  | 610              | 350   |
| Volume (cc.) of water after X minutes:             |      |                  |      |      |      |                  |       |
| 1 min.                                             | 7    | 4                | 5    | 3    | 3    | 9                | 120   |
| 2 min.                                             | 13   | 8                | 11   | 8    | 9    | 17               | 138   |
| 5 min.                                             | 46   | 35               | 39   | 29   | 34   | 56               | 147   |

<sup>1</sup> A blend of 22% sodium xylene sulfonate and 78% of C<sub>10</sub>-C<sub>13</sub> linear secondary alkyl benzene sulfonate.

<sup>2</sup> A blend containing:

(a) 20 parts of a C<sub>8</sub>-C<sub>10</sub> alkoxylated straight chain alcohol having an average of 10-12 alkoxy units of which three fourths are ethoxy and one fourth are propoxy.

(b) 80 parts of an aqueous solution of a C<sub>10</sub>-C<sub>13</sub> linear secondary alkyl benzene sulfonate wherein the solids content of the solution is 60% by weight.

Formulations 1, 3, 4 and 5 which represent embodiments of this invention generate at a faster rate an average of 47% more foam which is 53% more stable than the average of those produced by Formulations 2, 6 and 7 which are outside the scope of this invention.

## EXAMPLE II

30 The following example was conducted in accordance with the procedure set forth in Example I. The formulations were prepared using water of 500 p.p.m. hardness at 40° F.

TABLE II

| Formulation No.                                    | 8    | 9    | 10               | 11   | 12   | 13   | 14    | 15    |
|----------------------------------------------------|------|------|------------------|------|------|------|-------|-------|
| Average No. of carbons in alkyl chain              | 8.5  | 9.0  | 9.4              | 9.5  | 10.3 | 10.4 | 11.3  | 13.0  |
| Actual alkyl chain carbon range                    | 8-9  | 8-10 | ( <sup>1</sup> ) | 9-10 | 9-11 | 9-13 | 10-13 | 12-14 |
| Maximum carbon spread                              | 2    | 3    | 12               | 2    | 3    | 5    | 4     | 3     |
| Time (sec.) to generate specified amounts of foam: |      |      |                  |      |      |      |       |       |
| 500 cc.                                            | 21   | 15   | 45               | 14   | 15   | 19   | 110   | >120  |
| 600 cc.                                            | 29   | 22   | 76               | 20   | 21   | 30   | >120  | ----- |
| 700 cc.                                            | 70   | 40   | >120             | 32   | 46   | 51   | ----- | ----- |
| 800 cc.                                            | >120 | 115  | -----            | 100  | 95   | 115  | ----- | ----- |
| Total foam after 120 seconds                       | 725  | 800  | 620              | 800  | 825  | 800  | 520   | 275   |
| Volume (cc.) of water after X minutes:             |      |      |                  |      |      |      |       |       |
| 1 min.                                             | 6    | 5    | 10               | 5    | 3    | 3    | 25    | 150   |
| 2 min.                                             | 14   | 10   | 16               | 9    | 7    | 8    | 42    | 162   |
| 5 min.                                             | 64   | 42   | 51               | 36   | 27   | 33   | 108   | 154   |

As defined in Table I.

## EXAMPLE I

Frothing formulations were prepared utilizing 0.062% of the sodium salt of linear secondary alkyl benzene sulfonates in water of 100 p.p.m. hardness at 40° F. The carbon structures of the alkyl side chains are described in Table I. 160 cc. of each formulation was placed in a graduated cylinder and agitated on a Hamilton Beach #33 mixer. The time necessary to generate specific amounts of foam were noted. After 120 seconds the foam was transferred to a one liter graduated cylinder and the volume of drained water was recorded at various times. 60 made.

50 Formulations 8, 9, 11, 12 and 13 which represent embodiments of this invention generate at a faster rate an average of 68% more foam which is 36% more stable than the average of those produced by Formulations 10, 14 and 15 which are outside the scope of this invention.

## EXAMPLE III

The following example was conducted in accordance with the procedure set forth in Example I. The formulations were prepared with 500 p.p.m. water at 40° F. Five percent gypsum was added after the formulations were

TABLE III

| Formulation No.                                    | 16   | 17   | 18               | 19               | 20    | 21    | 22    | 23               |
|----------------------------------------------------|------|------|------------------|------------------|-------|-------|-------|------------------|
| Average No. of carbons in alkyl chain              | 8.5  | 9.0  | 9.4              | 10.0             | 10.3  | 10.4  | 11.3  | 11.3             |
| Actual alkyl chain carbon range                    | 8-9  | 8-10 | ( <sup>1</sup> ) | ( <sup>2</sup> ) | 9-11  | 9-13  | 10-13 | ( <sup>2</sup> ) |
| Maximum carbon spread                              | 2    | 3    | 12               | 8                | 3     | 5     | 4     | 4                |
| Time (sec.) to generate specified amounts of foam: |      |      |                  |                  |       |       |       |                  |
| 500 cc.                                            | 14   | 15   | >120             | 41               | 28    | 32    | >120  | >120             |
| 600 cc.                                            | 21   | 27   | -----            | 120              | 80    | 100   | ----- | -----            |
| 700 cc.                                            | 44   | 51   | -----            | >120             | >120  | >120  | ----- | -----            |
| 800 cc.                                            | >120 | 111  | -----            | -----            | ----- | ----- | ----- | -----            |
| Total foam after 120 seconds                       | 780  | 810  | 300              | 600              | 650   | 610   | 300   | 250              |
| Volume (cc.) of water after X minutes:             |      |      |                  |                  |       |       |       |                  |
| 1 min.                                             | 6    | 5    | 152              | 11               | 10    | 10    | 152   | 155              |
| 2 min.                                             | 15   | 11   | 158              | 27               | 22    | 27    | 156   | 158              |
| 5 min.                                             | 60   | 42   | 159              | 91               | 73    | 91    | 158   | 158              |

<sup>1</sup> and <sup>2</sup> as defined in Table I.

<sup>3</sup> A blend containing 27% of C<sub>6</sub>-C<sub>7</sub> and 73% of C<sub>10</sub>-C<sub>13</sub> linear secondary alkyl benzene sulfonates.

Formulations 16, 17, 19, 20 and 21 which represent embodiments of this invention generate at a faster rate an average of 144% more foam which is 55% more stable than the average of those produced by Formulations 18, 22 and 23 which are outside the scope of this invention.

## EXAMPLE IV

The following example was conducted in accordance with the procedure set forth in Example I. The formulations were prepared using water at 120° F. and 100 p.p.m. hardness.

Formulations 30, 31, 32, 33 and 34 which represent embodiments of this invention generate at a faster rate an average of 97% more foam which is 22% more stable than the average of those produced by Formulations 35 and 36 which are outside the scope of this invention.

## EXAMPLE VI

The following example was conducted in accordance with the procedure set forth in Example I. The tests were performed with water at 120° F., 500 p.p.m. hardness, and containing an additional 5% by weight gypsum.

| Formulation No.                                    | 37  | 38   | 39               | 40   | 41   | 42   | 43    | 44               |
|----------------------------------------------------|-----|------|------------------|------|------|------|-------|------------------|
| Average No. of carbons in alkyl chain              | 8.5 | 9.0  | 9.4              | 9.5  | 10.3 | 10.4 | 11.3  | 11.3             |
| Actual alkyl chain carbon range                    | 8-9 | 8-10 | ( <sup>1</sup> ) | 9-10 | 9-11 | 9-13 | 9-13  | ( <sup>2</sup> ) |
| Maximum carbon spread                              | 2   | 3    | 12               | 2    | 3    | 5    | 4     | 4                |
| Time (sec.) to generate specified amounts of foam: |     |      |                  |      |      |      |       |                  |
| 500 cc.                                            | 19  | 21   | >120             | 19   | 33   | 38   | >120  | >120             |
| 600 cc.                                            | 26  | 25   | -----            | 32   | 41   | 48   | ----- | -----            |
| 700 cc.                                            | 40  | 39   | -----            | 46   | 80   | 87   | ----- | -----            |
| 800 cc.                                            | 80  | 71   | -----            | 75   | >120 | >120 | ----- | -----            |
| Total foam after 120 seconds                       | 850 | 880  | 300              | 900  | 775  | 735  | 275   | 250              |
| Volume (cc.) of water after X minutes:             |     |      |                  |      |      |      |       |                  |
| 1 min.                                             | 20  | 11   | 153              | 12   | 14   | 22   | 153   | 155              |
| 2 min.                                             | 49  | 33   | 156              | 32   | 42   | 57   | 156   | 157              |
| 5 min.                                             | 118 | 102  | 158              | 99   | 112  | 126  | 158   | 157              |

<sup>1</sup> and <sup>2</sup> as defined in Table I.

TABLE IV

| Formulation No.                                    | 24  | 25   | 26   | 27   | 28   | 29               |
|----------------------------------------------------|-----|------|------|------|------|------------------|
| Average No. of carbons in alkyl chain              | 8.5 | 9.0  | 9.5  | 10.3 | 10.4 | 11.3             |
| Actual alkyl chain carbon range                    | 8-9 | 8-10 | 9-10 | 9-11 | 9-13 | ( <sup>2</sup> ) |
| Maximum carbon spread                              | 2   | 3    | 2    | 3    | 5    | 4                |
| Time (sec.) to generate specified amounts of foam: |     |      |      |      |      |                  |
| 500 cc.                                            | 27  | 16   | 13   | 12   | 18   | 65               |
| 600 cc.                                            | 31  | 20   | 16   | 14   | 22   | 77               |
| 700 cc.                                            | 51  | 29   | 20   | 18   | 28   | >120             |
| 800 cc.                                            | 120 | 61   | 34   | 29   | 46   | -----            |
| Total foam after 120 seconds                       | 800 | 900  | 930  | 920  | 915  | 660              |
| Volume (cc.) of water after X minutes:             |     |      |      |      |      |                  |
| 1 min.                                             | 12  | 8    | 9    | 5    | 7    | 13               |
| 2 min.                                             | 33  | 23   | 23   | 18   | 20   | 27               |
| 5 min.                                             | 114 | 91   | 87   | 71   | 77   | 86               |

<sup>2</sup> As defined in Table I.

Formulations 24, 25, 26, 27 and 28 which represent embodiments of this invention generate at a faster rate an average of 34% more foam than Formulation 29 which is outside the scope of this invention.

## EXAMPLE V

The following example was conducted in accordance with the procedure set forth in Example I. The formulations were prepared using water at 120° F. with 500 p.p.m. hardness.

TABLE V

| Formulation No.                                    | 30  | 31   | 32   | 33   | 34   | 35    | 36    |
|----------------------------------------------------|-----|------|------|------|------|-------|-------|
| Average No. of carbons in alkyl chain              | 8.5 | 9.0  | 9.5  | 10.3 | 10.4 | 11.3  | 13.0  |
| Actual alkyl chain carbon range                    | 8-9 | 8-10 | 9-10 | 9-11 | 9-13 | 10-13 | 12-14 |
| Maximum carbon spread                              | 2   | 3    | 2    | 3    | 5    | 4     | 3     |
| Time (sec.) to generate specified amounts of foam: |     |      |      |      |      |       |       |
| 500 cc.                                            | 25  | 15   | 13   | 15   | 21   | 83    | >120  |
| 600 cc.                                            | 29  | 18   | 15   | 18   | 25   | 96    | ----- |
| 700 cc.                                            | 50  | 26   | 21   | 25   | 34   | >120  | ----- |
| 800 cc.                                            | 90  | 48   | 31   | 36   | 53   | ----- | ----- |
| Total foam after 120 seconds                       | 810 | 900  | 930  | 900  | 900  | 650   | 250   |
| Volume (cc.) of water after X minutes:             |     |      |      |      |      |       |       |
| 1 min.                                             | 22  | 7    | 7    | 8    | 8    | 15    | 152   |
| 2 min.                                             | 60  | 25   | 22   | 22   | 21   | 33    | 155   |
| 5 min.                                             | 138 | 95   | 88   | 82   | 86   | 95    | 157   |

<sup>1</sup> and <sup>2</sup> as defined in Table I.

Formulations 37, 38, 40, 41 and 42 which represent embodiments of this invention generate at a faster rate an average of 200% more foam which is 30% more stable than the average of those produced by Formulations 39, 43 and 44 which are outside the scope of this invention.

## EXAMPLE VII

Gypsum slurries are prepared by agitating 100 parts of gypsum in 100 parts water. 0.25 part of potassium sulfate and 1.0 part starch are added as an accelerator and retarder respectively. 0.03 part of frothing Formulation Numbers 1, 3, 4 and 5 from Table I are agitated until foams having a density of about 12 lbs./ft.<sup>3</sup> are produced. These foams are then stirred into the various gypsum slurries. The slurries are then deposited between two layers of paper. The sheets are then cured at 300° F. until the free water has evaporated and the gypsum has set. The resultant boards are light in weight and have uniform density characteristics.

We claim:

- In the production of gypsum board comprising the steps of preparing a fluid gypsum slurry containing a froth, depositing the slurry between two impervious barriers and heating the slurry to evaporate the water and set the gypsum, the improvement which comprises utilizing as the frothing agent an alkyl benzene sulfonate having a linear secondary alkyl side chain with an average carbon content ranging from 8.5 to 10.5 and a maximum carbon number spread of eight carbons.
- A method according to claim 1 wherein the alkyl benzene sulfonate is utilized in amounts ranging from 0.01 to 0.1 per 100 parts gypsum.
- A method according to claim 1 wherein the alkyl benzene sulfonate has an average carbon number ranging from 9.5 to 10.5.
- A method according to claim 1 wherein the alkyl benzene sulfonate has a maximum carbon number spread of 5 carbon atoms.
- A method according to claim 1 wherein the alkyl benzene sulfonate is an alkali metal salt.

6. A method according to claim 5 wherein the alkali metal is sodium.

7. A method according to claim 1 wherein the froth is first prepared and then incorporated into the gypsum slurry.

8. A method according to claim 1 wherein the improvement comprises utilizing the sodium salt of an alkyl benzene sulfonate having a linear secondary alkyl side chain with an average carbon content ranging from 9.5 to 10.5 and a maximum carbon number spread of five carbon atoms.

**References Cited****UNITED STATES PATENTS**

2,913,346 11/1959 Hoffman ----- 106—111  
3,359,146 12/1967 Lane et al. ----- 106—111

5 JAMES E. POER, Primary Examiner

U.S. Cl. X.R.

10 106—112, 113, 114; 156—43